

## UNITED STATES PATENT OFFICE.

MATTHEW GREEN, OF DETROIT, AND HOBART H. WILLARD, OF ANN ARBOR, MICHIGAN, ASSIGNORS TO PARKER RUST-PROOF COMPANY, OF DETROIT, MICHIGAN, A CORPORATION OF MICHIGAN.

## PROCESS OF RUST PROOFING AND ARTICLES PRODUCED THEREBY.

No Drawing.

Application filed May 10, 1926. Serial No. 108,162.

This invention relates to a process of rust-proofing iron articles and to the articles rust-proofed in this manner.

More particularly, the invention relates to producing on the surface of iron articles a coating of phosphates which are insoluble in water, and to the articles coated in this manner.

The process of rust-proofing iron articles by producing thereon a coating of insoluble phosphates is well-known. While other materials have been used to some extent, the coatings which have been produced have been essentially phosphates of iron. Analysis shows that, while other phosphates are present to some extent, the major portion of the coating consists of ferrous monohydrogen phosphate. This particular phosphate is slightly soluble and, therefore, does not furnish complete protection against rusting.

It has been discovered that, when manganese dihydrogen phosphate is present in the rust-proofing bath in considerable proportions relatively to the other materials in the bath, a considerable portion of the coating consists of phosphate of manganese. The exact composition of the different phosphates in such a coating is very difficult to determine, but it has been discovered that, when a considerable percentage of manganese is present in such a coating, the proportion of phosphorus to metal in the coating more nearly approaches that present in the normal phosphate than that present in the monohydrogen phosphate. The exact proportion may be varied by many conditions, but the following examples may be mentioned in order to bring out clearly the intended distinction. When the coating contains iron and manganese atoms in about the ratio of two to one, the ratio of the metal to phosphorus is a trifle greater than that which would result from the coating being one-half monohydrogen phosphate and one-half normal phosphate. With manganese forming about one-half of the metal in the coating, the proportion of metal in the coating to phosphorus in the coating was found to indicate a proportion of approximately 6/7 normal phosphate and 1/7 monohydrogen phosphate. In the monohydrogen phosphate these atoms of metal and phosphorus are in

the ratio of 1 to 1, while in the normal phosphate the ratio is 3 to 2. Analyses of coatings containing iron and manganese in the proportion of 2 to 1 have shown an atomic proportion of 5 to 4 of metal to phosphorus, and similarly a proportion of 1 to 1 in the metals has shown a proportion of 1.4+ to 1 of metal to phosphorus.

Normal phosphate is much less soluble than monohydrogen phosphate, and corrosion tests corroborate the analyses described above. That is, coatings comparatively high in manganese and apparently high in normal phosphate are found to be much more resistant to rusting than coatings consisting largely of monohydrogen phosphate.

While this effect is gradually increased with the increase of manganese in the coating, it appears that the proportion of normal phosphate is increased more rapidly than the proportion of manganese, and that a proportion of manganese amounting to one-half as much as the iron in the coating is decidedly effective in increasing the quality of the coating, but that a percentage of manganese equaling that of the iron in the coating produces a very much more resistant coating. While beneficial results may be obtained from our invention by having present in the coating an amount of manganese equal to one-half of the iron in the coating, it is preferable to have at least as much manganese as iron in the coating in order to obtain a protective layer which is substantially normal phosphate.

It has been found that, where manganese dihydrogen phosphate and ferrous dihydrogen phosphate are present in a rust-proofing solution, the manganese phosphate being less than the ferrous phosphate, there is a selective action which results in producing in the coating a larger proportion of manganese than there is in solution in the bath. For example, one-third as much manganese as iron in a bath may result in one-half as much manganese as iron in the coating, while approximately one-half as much manganese as iron in the bath will produce approximately as much manganese as iron in the coating. It will be understood that many conditions alter these proportions to some extent, and that the proportions given above are for purposes of illustration and

are not given as being fixed ratios under all circumstances.

It follows from the above that the desired coating should contain at least one-half as much manganese as iron, and that for this purpose the bath should contain at least one-third as much manganese dihydrogen phosphate as it contains of ferrous dihydrogen phosphate.

10 There are several ways in which a bath of the desired composition may be obtained. Some of these ways will be described.

If manganese dihydrogen orthophosphate is dissolved in water, and the water boiled 15 for some time, a portion of the phosphate is precipitated as an insoluble phosphate and some free acid is liberated. We have found that from seven to seventy pounds of the said phosphate dissolved in one hundred twenty-five gallons of water and boiled as described will produce a satisfactory rust-proofing solution, twenty to twenty-five pounds being the preferred amount. When an iron article, or an article having a surface 20 containing iron, is immersed in such a solution, the formation of a rust-proofing coating begins at once. There is no preliminary pickling of the work to bring the solution into balance, such as necessarily 25 results where free acid is added to the bath and where iron must be dissolved from the work to bring the solution into balance, and the articles do not lose appreciably in weight or measurably in size. Nevertheless, 30 in the process of forming the coating, a certain amount of the iron is dissolved in the bath. Some of this is fixed as insoluble phosphates in coating, some of it forms insoluble phosphates which are deposited as 35 sludge, and part of it remains as ferrous dihydrogen phosphate dissolved in the bath. It will be readily understood that more of the phosphate radicals are in combination with a given amount of manganese in the 40 dihydrogen phosphate than there are in the insoluble coating and, therefore, the phosphate introduced into the bath introduces sufficient phosphate radicals to form the phosphates of iron mentioned above.

45 If the bath is used continuously for rust-proofing purposes for a considerable time, it constantly becomes less rich in manganese and richer in iron, reference being had to these materials dissolved in the bath in the form of dihydrogen phosphate. When the 50 bath is replenished by an additional amount of manganese phosphate, the proportion of manganese to iron is increased, but is not brought back to the proportion which it had originally. The proportion of iron in the bath continues to increase until it reaches a certain percentage in proportion to the maximum acidity. Thereafter the iron in the bath seems 55 to remain approximately constant, whereas 60 the manganese and acid are increased when

the bath is replenished and are gradually reduced as work is coated. The reason for the increase in iron up to a certain point with no further increase has not been ascertained, but the fact has been discovered.

If replenishing is delayed and rust-proofing is continued until the proportion of manganese and of free acid in the bath is relatively low, the proportion of iron to manganese is greatly increased. That is, if a bath which has reached a substantially constant iron content is replenished with manganese phosphate, it may be easily brought up to a point where the manganese will be more than half as much as the iron 80 in the bath, but as this bath is used for rust-proofing purposes the manganese may be almost completely exhausted from the bath before the deposition of a coating will cease. In such a case, the coating last formed is principally ferrous monohydrogen phosphate. By replenishing at comparatively short intervals, the amount of manganese in the bath may be kept above one-third as much as the iron, with a result 85 of producing more normal phosphate than monohydrogen phosphate in the coating. The strength of the rust-proofing solution may be varied considerably and still rust-proof effectively. However, as the amount 90 of iron in the bath seems to be approximately relative to the maximum acidity of the bath, it is preferable to replenish the bath to bring it each time to approximately 95 the same strength. In this way the proportion of manganese to iron is increased to the highest practicable amount at each replenishment.

Theoretically, the best results would be obtained by replenishing the bath constantly so as to keep it at a substantially constant strength, as that would maintain the proportion of manganese in the bath at its highest point continuously. However, there are some objections to replenishing during the time of rust-proofing in the same bath, and the next best results are obtained by replenishing after each load. As it is desirable to allow some time for the bath to become uniform after each replenishment, there is some delay due to replenishing after each load. Satisfactory results may be obtained by replenishing after every other load. In general, it may be stated that the manner and frequency of replenishment will depend to some extent upon the quality of the coating desired. For the highest quality of coating, the bath should be kept as nearly as is practicable to the highest available proportion of manganese. Sometimes the coating produced with a less percentage of manganese is entirely sufficient for the desired purposes, and in such cases less care is required in maintaining the bath with a uniformly high manganese content.

While the preferred method of replenishing the bath is by adding a material consisting essentially of manganese dihydrogen phosphate, it will be understood that other methods may be used for obtaining the desired bath. This invention relates more especially to the bath which is desired, to the manner of replenishment, and to the coating produced. Various modifications may be made within the scope of the appended claims.

What we claim is:

1. Iron or steel or articles composed or having a surface of iron or steel furnished with a coating or deposit of phosphates of iron and of manganese, there being at least one-half as much manganese as iron in the coating.
2. Iron or steel or articles composed or having a surface of iron or steel furnished with a coating or deposit of phosphates of iron and of manganese, there being in the coating more than six atoms of the metal to five atoms of phosphorus.
3. A method of rust-proofing articles of iron or having a surface of iron or steel which consists in forming a dilute solution of phosphoric acid and dihydrogen phosphates of iron and manganese, there being at least one-third as much manganese as iron in the solution and there being sufficient dihydrogen phosphates in the solution in proportion to the free acid to rust-proof articles without reducing the weight

thereof, placing iron or steel articles in the solution and maintaining the solution hot until the articles are rust-proofed.

4. The method of rust-proofing articles of iron or having a surface of iron or steel which consists in forming a dilute solution of phosphoric acid and dihydrogen phosphates of iron and manganese, there being at least one-third as much manganese as iron in the solution and there being sufficient dihydrogen phosphates in the solution in proportion to the free acid to rust-proof articles without reducing the weight thereof, placing iron or steel articles in the solution and maintaining the solution hot until the articles are rust-proofed, introducing other articles into the bath and repeating the process and adding to the solution from time to time materials which maintain the amount of manganese in the solution above one-third the iron in the solution.

5. A solution for rust-proofing purposes containing dihydrogen phosphates of manganese and iron and free acid, the phosphates being in sufficient amounts so as to rust-proof an immersed iron article without significant loss of weight and the manganese in the dissolved phosphates being more than one-third as much as the iron in the dissolved phosphates.

In testimony whereof we have hereunto signed our names to this specification.

HOBART H. WILLARD.  
MATTHEW GREEN.